

Sept. 23, 1941. A. F. P. J. CLAASSEN ET AL

2,256,860

METHOD AND DEVICE FOR MAKING ALUMINUM ELECTRODES

Filed April 26, 1939



Fig. 1.



Fig. 2.

INVENTORS  
A. F. P. J. CLAASSEN and  
J. D. de Vries

BY *W. F. Ondroth.*

ATTORNEY

## UNITED STATES PATENT OFFICE

2,256,860

METHOD AND DEVICE FOR MAKING  
ALUMINUM ELECTRODES

Anthony Frederik Peter Johannes Claassen and  
Johan Dirk de Vries, Eindhoven, Netherlands,  
assignors, by mesne assignments, to Hartford  
National Bank and Trust Company, Hartford,  
Conn., as trustee

Application April 26, 1939, Serial No. 270,266  
In Germany May 19, 1938

## 5 Claims.

(CL 148—8)

Our invention relates to a method and device for increasing the active surface area of aluminum electrodes, particularly electrodes for electrolytic condensers, by chemical agency.

The term "chemical agency" is to be understood to include the usual chemical cauterization or etching, as well as cauterization or etching by electrochemical agency.

To increase the active surface area of aluminum electrodes it is known to cauterize them, for example in hydrochloric acid, and in such cases the temperature of the cauter bath employed was usually about 20 to 25° C., but higher temperatures have been suggested. In view of the generally recognized fact that the rapidity of a reaction is materially increased with an increase of temperature, one skilled in the art had come to the conclusion that the temperature of the cauter bath should be as high as possible to insure a sufficiently quick cauterizing effect. For example, the British Patent 448,163 suggests that the temperature of the cauter solution be maintained at the boiling point, i. e. at approximately 100° C.

We have found that when the cauter solution is maintained at such relatively high temperatures, it is impossible to obtain with uniformity a material increase in the active surface area. More particularly, although the usual methods of cauterization make it possible to obtain with regular results an electrode which gives a capacity of from four to eight times that obtained with an electrode having smooth surfaces, it is difficult, if not impossible, to obtain with such methods a greater surface increase in mass production.

The main object of our invention is to produce a greater increase in the active surface area of an aluminum electrode by chemical agency.

A further object is to provide a method of increasing the active surface area with which uniform results can be obtained in mass production.

Further objects of our invention will appear as the description progresses.

According to the invention, we maintain the solution used for the cauterization at a temperature which is below 8° C. and above the freezing point of the solution.

By maintaining the temperature of the cauter solution within the above-mentioned range, the duration of the cauterization process is increased, but quite unexpectedly the increase in the active surface area is much greater than when the solution is maintained at the higher temperatures

usually employed. Furthermore, we have found that such a material increase is not obtained by cooling the solution with comparatively cold tap water.

5 We have found that the improved results obtained by the present invention are due solely to the decrease in temperature of the solution. Although one might think that a decrease in concentration of the solution would have the same 10 effect, this is not the case in practice because the increase in the active surface is obtained only if the temperature of the solution is maintained within the above-mentioned range.

In order that the invention may be more clearly understood and readily carried into effect, we shall describe the same in more detail with reference to the accompanying drawing, in which, Figure 1 is a sectionized side view of an apparatus in which the cauter liquid is indirectly cooled, and

Fig. 2 is a sectionized view of an apparatus in which the cauter solution is directly cooled.

The apparatus shown in Figure 1 comprises a suitable container 1 filled with a cauter solution 10, for example a solution consisting of hydrochloric acid and a small addition of aluminum chloride. Container 10 is partly immersed within a cooling liquid 3, such as a solution of salt in water, contained in a second container 2. A suitable refrigerant supplied from a source (not shown), is circulated through the cooling coil 4 and serves to cool the liquid 3 and thus the solution 10.

To obtain a regular circulation of the liquid 3 we provide two stirrers 5 which rotate in opposite directions and circulate liquid 3 in the direction indicated by the arrows. In the present instance the cauter solution is maintained at a temperature between 2° C. and 8° C. and preferably at a temperature of about 5–6° C.

In Figure 2 a container 11 is filled with a cauter solution 7, also containing a solution of hydrochloric acid. The solution 7 is maintained at a temperature below 8° C. and above its freezing point, for instance at a temperature of about 6° C., by a cooling coil 6 through which a suitable refrigerant, such as glycerine dissolved in water, supplied from a refrigerator 8 is circulated by a pump 9.

50 The method according to the invention may be used independently or in conjunction with known methods for obtaining a highly enlarged surface area in electrodes for electrolytic condensers. For example, the present method may be used for electrodes consisting of aluminum

whose copper percentage is kept below a certain value, for instance 0.05%, to improve the cauterizing effect; also for types of aluminum having a very small crystal-grain size, for instance 1 micron.

The advantage of the method according to the invention over prior-art methods will clearly appear from the following comparison test.

Electrodes having a geometric or contour surface area of about 100 sq. cms. were made from aluminum having a purity of about 99.85%. The cauter bath used consisted of a solution of approximately 9% hydrochloric acid in distilled water, to which was added a quantity of aluminum chloride ( $AlCl_3$ ) corresponding to a 15 quantity of 20 grams of aluminum per liter. According to tests, this proved to be a concentration yielding the largest surface increase. The temperature of the cauter bath was maintained at about 20° C. and the electrodes were cauterized for 1½ hours in this solution and then formed to a voltage of 500 volts. We found that the electrodes had a capacity of from 8 to 9 microfarads, and these results could be uniformly produced in mass production. With a longer duration of cauterizing the capacity did not increase further.

In accordance with the invention, the above tests were repeated under the same conditions except that the cauter bath was maintained at a temperature of about 6° C. and the duration of cauterizing was increased to 3-3½ hours. For electrodes having the same contour surface area and with the same formation process a capacity of 14 to 15  $\mu$ f was now obtained.

Even when the surface enlargements obtained will slightly vary through various influences, it is yet possible to obtain in a reproducible manner an improvement of the active factor of surface increase which materially exceeds 50% with regard to the factors obtained heretofore.

It should be noted that because of the reduction in the geometric dimensions of the electrodes, the method according to the invention results in an increase of the series resistance in

a condenser, but this difficulty can be overcome by using the proper electrolyte and by mounting the electrodes so as to make the current path through the electrolyte as small as possible.

5 We wish it to be understood that we do not wish to be limited to the exact details described, because obvious modifications will occur to a person skilled in the art.

What we claim is:

10 1. A method of increasing the active surface of an aluminum electrode by chemical agency, comprising the steps of placing the electrode in an etching solution, and maintaining the solution at a temperature above its freezing temperature and below 8° C.

20 2. In the treatment of aluminum electrodes with an etching solution to increase the surface area by chemical agency, cooling the solution to a temperature above its freezing temperature and below 8° C.

25 3. A method of increasing the active surface of an aluminum electrode by chemical agency, comprising the steps of placing the electrode in an etching solution containing hydrochloric acid, and maintaining the solution at a temperature above its freezing temperature and below about 8° C.

30 4. A method of increasing the active surface of an aluminum electrode by chemical agency, comprising the steps of placing the electrode in an etching solution of hydrochloric acid and aluminum chloride, and maintaining the solution at a temperature above its freezing temperature and below about 8° C.

35 5. A method of increasing the active surface of an aluminum electrode by chemical agency comprising the steps of placing the electrode in a 9% hydrochloric acid aqueous etching solution, and maintaining the etching solution at a temperature above its freezing temperature and below about 8° C.

ANTHONY FREDERIK PETER  
JOHANNES CLAASSEN.  
45 JOHAN DIRK DE VRIES.